

## 1

3,067,138

**FUEL AND LUBRICATING OIL COMPOSITIONS**  
Christian Jahan, Gruchet-le-Valasse, and Michel Tourrier, Notre-Dame-de-Gravenchon, France, assignors to Esso Research and Engineering Company, a corporation of Delaware  
No Drawing. Filed Oct. 6, 1958, Ser. No. 765,280  
Claims priority, application France Oct. 10, 1957  
17 Claims. (Cl. 252—54)

The present invention relates to improved fuel and lubricating oil compositions for internal combustion engines e.g. two-stroke and four-stroke engines.

It is well-known that the accumulation of deposits in the combustion chambers of internal combustion engines brings about a considerable increase in the octane number requirement of the engine. In particular it has been found that vehicles after initial running, normally require petrol with an increase octane number over that required to begin with. Deposits formed in the engine are also accompanied by loss of power output, which may be as much as 10% or more. Further, fouling of the plugs occurs which can lead to stoppage on pre-ignition.

Certain additives, such as lead compounds, which are employed to raise the octane number of the fuel employed in the engine also play their part in producing deposits in the combustion chamber. This may occur even if detergents are used. Furthermore, the operation of internal combustion engines is also interfered with by carburetor icing. This occurs in particular when the engine is idling in a humid atmosphere having a temperature of less than 16° C., and can result in stalling of the engine due to fuel starvation.

Two-stroke engines are at present generally lubricated with detergent or non-detergent lubricating oils, the oils being blended with the fuel. These compositions generally produce deposits in two-stroke engines which cause spark plug fouling, marked wearing of the valves and of the crank shaft, progressive obstruction of the exhaust port, and loss of power.

It has now been discovered that by the addition of certain additives, hereinafter described, to fuel or lubricating oils, many of the above disadvantages may be overcome.

The additives used in the compositions according to the present invention are halogenated aliphatic compounds containing one or more alcohol groups, ether groups, aldehyde groups, or ketone groups, or mixtures of two or more of such groups. The compounds may have straight or branched chain structures and may be saturated or unsaturated. Chlorinated compounds are especially preferred.

Examples of suitable compounds are those of the following general formulae:

(1) CHLORINATED ALCOHOLS AND ETHERS



where X is halogen, R<sub>1</sub> and R<sub>2</sub> are the same halogen as X, hydrogen or an alkyl group, R<sub>3</sub> is an alkylene group, R<sub>4</sub> is hydrogen or an alkyl group, R<sub>5</sub> is hydrogen or an aliphatic group, and n is 0 or 1. The radicals R<sub>1</sub>, R<sub>2</sub>, R<sub>3</sub>, R<sub>4</sub> and R<sub>5</sub>

## 2

may contain such constituents as sulphydril, alkoxy and nitrile groups.

(2) CHLORINATED ALDEHYDES AND KETONES



where X is halogen, R<sub>1</sub> and R<sub>2</sub> are the same halogen as X, or hydrogen or an aliphatic group, and R<sub>3</sub> is hydrogen, a methyl group, or a chloromethyl group.

In Formula 1, R<sub>5</sub> is preferably a C<sub>1</sub> to C<sub>20</sub> alkyl group, particularly a C<sub>4</sub> to C<sub>12</sub> alkyl group. The preferred compounds in this class are those of formula



where R<sub>5</sub> is C<sub>1</sub> to C<sub>20</sub> alkyl.

Examples of these compounds are chloral ethyl alcoholate, and chloral iso-amyl alcoholate. Compounds in which R<sub>5</sub> is a C<sub>8</sub> or higher alkyl radical may also be used, and have the advantage of being liquid, but insoluble in water. This makes the compounds easier to mix with the fuel and lessens the risk of having the additive content of the fuel lessened in the event of storage in the presence of water.

Another preferred compound falling within Formula 1 is chloral hydrate:



Examples of compounds of Formula 2 are chloral, CCl<sub>3</sub>.CHO, compounds of formula R.CCl<sub>2</sub>.CHO, where R is an aliphatic hydrocarbon radical, and chlorinated acetones, e.g. Cl.CH<sub>2</sub>.CO.CH<sub>3</sub> and Cl.CH<sub>2</sub>.CO.CH<sub>2</sub>.Cl.

The fuel oil may be a gasoline, e. g. having a final boiling point of up to 300° C. In fuel compositions the additive may conveniently be present in proportions of from 0.001% to 1%, particularly 0.01% to 0.2% by weight based on the total composition.

The additives hereinbefore described may also be incorporated in lubricating oils to produce compositions according to the present invention. Such oils may be paraffinic or naphthenic in nature, and are preferably solvent-treated oils. The oils may have a viscosity of 76 to 329 cs. at 50° C. Lubricating oils intended for use in two-stroke engines may conveniently be diluted with an oil of lower viscosity, e.g. kerosene, spindle oil, or gas oil to facilitate admixture with the fuel. Thus the viscosity of the lighter oil may be between 1 and 22 cs. at 50° C. Such a mixture may contain between 50 and 70% of diluent oil.

The quantity of the additive added to the lubricating oil may be a minor proportion e.g. between 0.1 and 50%, preferably between 0.2 and 10% by weight, based on the total lubricating oil (i.e. excluding any diluent present). From 2 to 10% of the lubricating oil may be blended with fuel for use in a two-stroke engine and the amount of additive in this total oil/fuel blend may be 0.02 to 0.1%, preferably 0.05 to 0.1%.

The lubricating oil composition may also be used in the top cylinder lubrication of four-stroke engines, in which

case the lubricating oil may be a low boiling petroleum oil or a synthetic oil, preferably with a viscosity of 5 to 30 cs. at 50° C. In this application, the quantity of additive added to the oil may be from 0.1 to 50%, preferably 0.5 to 10% by weight in relation to the lubricating composition. These lubricants may be blended with the fuel in proportions of 0.1 to 1%.

The compositions of this invention may also contain various optional ingredients, e. g. oiliness agents, resin (gum) solvents, anti-knock agents, anti-oxidants, anti-rust agents, metal deactivators and scavengers.

The invention may be illustrated by the following examples.

#### Example 1

Bench tests were carried out on a Renault engine having the following characteristics:

Number of cylinders ..... 4.  
Bore and stroke in mm. ..... 58 x 80.  
Rated output in H.P. ..... 5.  
Maximum output in H.P. ..... 26.5 at 4,250 r.p.m.  
Cylinder capacity in cc. ..... 845.  
Compression ratio ..... 7.25.

In the course of these tests, periods of operation each of 5½ hours followed one another as follows:

| Conditions of operation | Part I | Period of 5½ hours |          |  |
|-------------------------|--------|--------------------|----------|--|
|                         |        | Part II            | Part III |  |
| Time in hours           | 1½     | 2                  | 2        |  |
| Speed in r.p.m.         | 600    | 2,400              | 2,400    |  |
| Output in h.p.          | 0      | 7.2                | 7.2      |  |
| Temperature in °C.:     |        |                    |          |  |
| Water outlet            | 46±3   | 70±3               | 70±3     |  |
| Crank case oil          | 46±3   | 80±3               | 85±3     |  |

After a first draining carried out after 150 hours' running, draining was then carried out every 44 hours (viz.: every 8 periods).

The tests were carried out with a fuel with and without the addition of chloral ethyl alcoholate.



The fuel employed was a high-grade fuel having the following characteristics:

Density at 15° C. ..... 0.720.  
Final distillation point ..... 180° C.  
Lead tetraethyl ..... 0.45 cc./litre.  
Octane number (research method) ..... 90.  
Reid vapour pressure at 38° C. ..... 706 g./sq. cm.

The tests yielded the following results:

#### OCTANE NUMBER REQUIREMENT (MEASURED BY THE APPEARANCE OF TRACES OF PINKING)

|                          | Fuel alone | Fuel plus 0.4 g. chloral ethyl alcoholate per litre |
|--------------------------|------------|-----------------------------------------------------|
| Initially                | 71         | 71                                                  |
| After 210 hours' running | 81         | 77                                                  |
| Increase in demand       | 10         | 6                                                   |

#### Example 2

Road tests were carried out with two Renault cars ("Dauphine") one using the fuel alone, the other plus the additive according to the invention. These two cars were used together under normal driving conditions on the road, with the leading car regularly changed. The tests were commenced with cars whose engines were perfectly clean. After a certain number of kilometres, the octane number demand ceases to increase and attains a maximum which corresponds to a kind of engine balance.

The octane demand is measured by the traditional methods at the start and in the state of equilibrium.

These tests were conducted by using:

(1) A high-grade fuel containing more lead than the commercial high-grade fuels, so as to show the efficacy of the additive from the point of view of the elimination of deposits, and having the following characteristics:

Density at 115° C. ..... 0.722.  
Final distillation point ..... 181° C.  
Lead tetraethyl ..... 0.8 cc./litre.  
Octane number (research method) ..... 94.  
Reid vapour pressure at 38° C. ..... 500 g./sq. cm.

(2) The same high-grade fuel with the addition of 0.7 g. per litre chloral ethyl alcoholate.

The tests yielded the following results:

|                    | Octane number demand  |                                                                |
|--------------------|-----------------------|----------------------------------------------------------------|
|                    | High grade fuel alone | High grade fuel plus 0.7 g. chloral ethyl alcoholate per litre |
| Initially          | 70                    | 70                                                             |
| At equilibrium     | 85                    | 76                                                             |
| Increase in demand | 15                    | 6                                                              |

#### Example 3

Tests were carried out on the road under normal driving conditions with cars that had already run without their engines having been decarbonised.

These cars were supplied with the same high grade fuel as in Example 2 (i.e. a premium fuel whose TEL content was raised to 0.8 cc. per litre), plus 0.7 g. chloral ethyl alcoholate.

After 4000 km. the octane demand of the vehicle was measured to compare it with the initial demand.

| Type of vehicle  | Initial | Octane demand after 4,000 km. | Reduction |
|------------------|---------|-------------------------------|-----------|
| Versailles       | 70      | 64                            | 6         |
| Simca Aronde     | 76      | 74                            | 2         |
| Renault 4 H.P.   | 83.5    | 77                            | 6.5       |
| Renault Dauphine | 85      | 78                            | 7         |
| Renault Fregate  | 89      | 85                            | 4         |
| Peugeot 403      | 78      | 68                            | 10        |
| Citroen 2 H.P.   | 79      | 76.5                          | 2.5       |

This table shows the efficacy of the fuel improved according to the invention from the point of view of the lowering of the octane demand even when used for supplying a vehicle that has already run, without it being necessary to decarbonise the engine.

#### Example 4

Similar tests to those of Example 1, were carried out by using a fuel with and without the addition of chloral hydrate:



The fuel used was an ordinary motor spirit having the following characteristics:

Density at 15° C. ..... 0.726.  
Final point of distillation ..... 198° C.  
Lead tetraethyl ..... 0.5 cc./litre.  
Sulphur ..... 0.7%.  
Octane number (research method) ..... 80.1.  
Reid vapour pressure at 37.8° C. ..... 580 g. sq. cm.

Use was made of chloral hydrate in the form of an alcoholic solution: 375 g. chloral hydrate are dissolved in a litre of alcohol, e.g. ethyl alcohol. The quantity added



3. A fuel as defined by claim 1 wherein said R<sub>5</sub> contains from 4 to 12 carbon atoms.

4. A fuel as defined by claim 1 wherein said compound is present from 0.01 to 0.2% by weight of the total fuel composition.

5. A fuel as defined in claim 1 wherein X is a chlorine atom.

6. A gasoline fuel to which has been added between 0.001 and 1.0% by weight of chloral iso-amyl alcoholate.

7. A gasoline fuel to which has been added between 0.001 and 1.0% by weight of chloral ethyl alcoholate.

8. A gasoline fuel to which has been added between 0.001 and 1.0% by weight of chloral hydrate.

9. A gasoline fuel to which has been added between 0.01 and 0.2% by weight of chloral iso-amylate and between 2 and 10% by weight of a lubricating oil having a viscosity of about 305 cps. at 37.8° C.

10. A lubricating oil for use in internal combustion engines having a viscosity of between 76 and 329 cps. at 50° C. to which has been added between 0.2 and 10% by weight of a compound having the formula:



wherein X is a halogen atom and R<sub>5</sub> is selected from the group consisting of hydrogen and an alkyl group of from 1 to 20 carbon atoms.

11. A lubricating oil composition as defined by claim 10 wherein said R<sub>5</sub> contains from 4 to 12 carbon atoms.

12. A lubricating oil as defined by claim 10 wherein said oil has been diluted with from 50 to 70% by weight of a lubricating oil of between 1 and 22 cps. viscosity at 50° C.

13. A lubricating oil as defined by claim 10 wherein said oil is a solvent treated paraffinic oil.

14. A lubricating oil as defined by claim 10 wherein said oil is a solvent treated naphthenic oil.

15. A lubricating oil having a viscosity of between 76 and 329 cps. at 50° C. to which has been added between 0.2 and 10% by weight of chloral iso-amyl alcoholate.

16. A lubricating oil having a viscosity of between 76 and 329 cps. at 50° C. to which has been added between 0.2 and 10% by weight of chloral ethyl alcoholate.

17. A lubricating oil having a viscosity of between 76 and 329 cps. at 50° C. to which has been added between 0.2 and 10% by weight of chloral hydrate.

References Cited in the file of this patent

UNITED STATES PATENTS

|           |                |       |                |
|-----------|----------------|-------|----------------|
| 1,949,588 | Thomas         | ----- | Mar. 6, 1934   |
| 2,068,635 | Prutton        | ----- | Jan. 19, 1937  |
| 2,137,784 | Prutton et al. | ----- | Nov. 22, 1938  |
| 2,214,768 | Lincoln        | ----- | Sept. 17, 1940 |
| 2,262,019 | Lincoln et al. | ----- | Nov. 11, 1941  |
| 2,272,923 | Prutton        | ----- | Feb. 10, 1942  |
| 2,281,598 | Prutton        | ----- | May 5, 1942    |
| 2,569,122 | Adelson        | ----- | Sept. 25, 1951 |
| 2,849,304 | Lyben          | ----- | Aug. 26, 1958  |